

## UNITED STATES PATENT OFFICE.

HECTOR AMPHION BATTALIOU, OF CAPE TOWN, CAPE PROVINCE, SOUTH AFRICA.

## ROAD-MAKING MATERIAL.

No Drawing.

Application filed January 14, 1924. Serial No. 686,201.

The modern practice of macadamizing roads makes such work an enormous item in the municipal and Governmental expenditure of all countries. The highly destructive action of modern motor traffic requires a maximum of binding power in connection with all macadamizing operations. The binder herein set out results in tremendous consolidation and gives a swift and permanent hardening effect combined with an elasticity both to an extent absent in the far more expensive processes involved in modern cementation. Experimental research work has determined the percentages of the mixture hereinafter set out. The composition, subject to variations hereinafter set out, consists of:—

|                         | Percent: |
|-------------------------|----------|
| Quartz sand             | 37       |
| 20 Carbonate of calcium | 35       |
| Oxide of iron           | 15       |
| Silicate of aluminium   | 12       |
| Amorphous carbon        | 1        |
|                         | 100      |

This is a new combination, the result of experiment and analysis and varying between the percentages hereinafter set out. The above combination when put together from the raw materials produces the above effects.

The above composition may vary in practice within certain maxima and minima percentages subject to slight loss of efficiency as hereinafter set out.

The quartz sand set out above at the ideal percentage of 37% may vary in practice between 45% and 30%. The result of an excess of quartz sand over and above 45% is to make the composition too hard with failure to secure uniformity of mixture, resulting in lack of adequate consolidation, and lack of binding power. It must here be especially noted that of all dangers due to excessive variation from the ideal as above set out, the danger caused by an increase in the percentage of quartz sand is the most serious to efficiency. And for this purpose it is advisable, except under quite exceptional circumstances, not to exceed a total of 40%. If less than 30% of quartz sand is used, the composition loses too much of its capacity for mechanical friction grip on the sides of the stones forming the macadam, and the petrification ultimately set up by the inter-

action between the carbonate of calcium and the quartz sand will be definitely lessened, and the composition will lose in toughness, effectiveness and durability.

The carbonate of calcium set out above at the ideal percentage of 35% may vary in practice between 42% and 32%. The carbonate of calcium permits of less variation in quantity relative to its total percentage than the oxide of iron and in practice the percentages should be limited rather more carefully between 40% and 35% in order to be certain of efficiency. If the carbonate of calcium is reduced proportionately with the oxide of iron, this leaves too large a proportion of the remaining constituents. If the oxide of iron is used in a higher percentage than 20%, this tends to give excessive penetration and slight dessication of the carbonate of calcium by the oxide of iron, with a loss of toughness and resiliency. The converse observation as to the simultaneous increase of the carbonate of calcium obtained is that the total amount of the remaining materials would then be too small. The fundamental objection to any increase of brittleness or loss of resiliency as above set out, is that the road would then wear much quicker than when the limits of efficiency between 20% and 10% are observed.

The oxide of iron set out above at the ideal percentage of 15% may vary in practice between 20% and 10%, but these variations from the ideal in either direction tend to sacrifice that inherent toughness of the composition contributed to it by the oxide of iron. If these margins are exceeded in either direction, definite excessive brittleness sets in. In the case where oxide of iron is less than 10% of the mixture, it becomes in operation too brittle by reason of too large a comparative quantity of carbonate of calcium. The same relative comments as to the ratios of the carbonate of calcium and the oxide of iron apply here as set out above, with, of course, the incidence of these comments reversed.

It is an essential portion of this invention that the sum total of the quartz sand and the carbonate of calcium should, as a joint contribution to the composition, not exceed 60% and not less than 45%. Should they exceed, it would have to be at the expense of either the silicate of aluminium or the quartz sand, an undue absence of either of which

would have results indicated hereinafter. On the other hand, if the carbonate of calcium and the oxide of iron are present in less quantity the similar results indicated hereinafter caused by excess of the quartz sand or

the silicate of aluminium would result. As to the general proportions of the oxide of iron and the carbonate of calcium, each to each, the latter should exceed the former by 5 not less than twice the quantity nor more than four times, but in either case, as already stated, variation from the ideal will give a slight, although within the limits indicated, a not very material decrease in efficiency.

10 15 Silicate of aluminum set out above at the ideal percentage of 12% may vary in practice between 22% and 7%. The result of exceeding 22% in this case is that a tendency to crack, to undue plasticity and to undue retardation of consolidation develops. The result of putting in less than 7% is that the composition loses both in compressibility and compactness with the resulting loss of consolidating strength.

20 25 The carbon which is present in a relatively small quantity in this composition and which is set out above at the ideal percentage of 1% may vary from  $\frac{1}{4}\%$  to  $\frac{2}{3}\%$ . It must be amorphous and finely divided. More than 2% would result in a distinct loss of hardening effect. The absence of the carbon would result in delay in the consolidating action. The use of carbon in any other form interferes with the process of recrystallization that occurs when the above composition is put into practical application with water, but amorphous carbon is too soft to cause such interference.

30 35 40 45 This composition for its best practical application in the ideal form requires reduction to a fine powder, but consolidation sufficient for practical purposes can be obtained under the following circumstances. The quartz sand must not be crushed more than to a minimum of  $\frac{1}{16}$  inch or it will lose its frictional and interlocking value. The rest can vary from  $\frac{1}{4}$  inch downward but  $\frac{1}{16}$  inch is best for the whole composition as this will include in practice a considerable percentage of the other constituents actually reduced to powder.

50 55 60 To sum up, the invention a combination of well known materials conforming as a result of selection, quantitative analysis and calculation with the ideal composition above set out within the limits of variation above indicated.

65 70 75 This composition slightly deadens the noise usually associated with a macadamized road. The only condition with regard to the macadam used with this composition is that it shall not be capable of latent deterioration. In other words, any ordinary sound macadam will do.

A further feature of the invention consists in the process by which this composition is used in practice. The best result is obtained as follows.

Upon and all over the surface of the proposed road which has been roughly rolled after the ordinary levelling and rough smoothing required for the road, and of course only where the surface is not bog or otherwise unsuitable in its entirety for road-making or construction, a layer of  $3\frac{1}{4}$  inches of the composition is laid. This is covered by some 4 inches to  $4\frac{1}{2}$  inches of macadam with a maximum in case of need of 6 inches.

In practice  $4\frac{1}{2}$  inches should not be exceeded. This is rolled and another layer of  $3\frac{1}{4}$  inches of the composition is spread over the top. This is then watered and rolled again, watered and rolled again, and any surface faults of an obvious nature filled up with a little more of the composition. This road can be used within twelve hours having initial binding to hold the camber against heavy street traffic. This binding will increase with time during which it will improve with traffic. The results of this method are as follows:

The water will saturate the macadam from the top down carrying with it an intimate mixture of the composition laid above the macadam. On reaching the lower layer of the composition, it in part will draw this up to meet the upper layer, and carrying on downward will take portions of the lower layer into all latent fissures, consolidating every crack, weakness or hole in the lower or natural road prior to the arrival of traffic thereon. This system will therefore prevent creeping downhill of the finished roadway; prevent any lateral creeping away from the artificial hill or crown of the camber, consolidating such raw or natural crown underneath; provide a firm lower base which will effectually prevent the dropping out or displacement of the lower stones in the macadam by presenting to them a hard and solid foundation not penetrable by them; prevent any movement of any macadam stone whatsoever in the mass as laid, giving adequate support to all such points of individual stones in the macadam as would otherwise be calculated to crush under the vibration of heavy traffic, and ultimately to cause subsidence and surface potholes.

Owing to the margin required for consolidation of the ground below the lower layer of the composition (consolidation of which acts as a foundation, without extra expenditure, for the whole structure) the lower  $3\frac{1}{4}$  inch of the composition cannot be relied upon to rise under the influence of the water, except under an exceptionally heavy roller, more than 2 inches, wherefore

4½ inches is the maximum for best results. This means that if 8 inches or 9 inches of macadam is required to be used, the surplus of macadam over 4½ inches must be put on as a second layer above the second layer of the composition and a third layer of the composition must be superimposed thereon. In practice, one layer of 4½ inches of macadam laid with two layers of the composition as above set out, will be enough save in exceptional cases.

The characteristic features of the present invention are (1) the discovery of a new synthetic combination of well known materials readily obtainable, which combination conforms with the percentages above set out within the limits indicated and which, after reduction to a powder within the limits above set out and mixed and applied to roads as above set out, results in a hard, insoluble, consolidating, cementing mass, in other words, the discovery of a new and improved binder; and (2) a simple process of applying the said composition in layers so as to form not only a tough, resilient and tenacious road but also a secure foundation therefor.

What I claim is:

1. A binding material for macadam, comprising a mixture of approximately 37 per cent sand, 35 per cent calcium carbonate, 15 per cent iron oxide, and 12 per cent aluminium silicate, all the ingredients being in

the form of particles not exceeding ¼ inch in greatest dimension. 35

2. A composition for the construction of roads and like surfaces, comprising a mixture of at least 37 per cent quartz sand, about 35 per cent calcium carbonate, about 12 per cent aluminum silicate, and iron oxide in sufficient quantity to make with the calcium carbonate not more than 60 per cent nor less than 40 per cent of the mixture. 40

3. A composition according to claim 2, wherein the quartz sand is in the form of particles not exceeding ¼ inch in greatest dimension. 45

4. A composition for the construction of roads and like surfaces, comprising a mixture of about 37 per cent fine aggregate, about 35 per cent calcium carbonate, about 12 per cent aluminium silicate, and about 15 per cent iron oxide. 50

5. A composition for the construction of roads and like surfaces, comprising a mixture of about 37 per cent fine aggregate, about 35 per cent calcium carbonate, about 12 per cent aluminum silicate, iron oxide in sufficient quantity to make with the calcium carbonate not more than 60 per cent nor less than 40 per cent of the mixture, and about 1 per cent amorphous carbon. 55

In testimony whereof I have signed my name to this specification.

HECTOR AMPHION BATTALIOU.